

# UNITED STATES PATENT OFFICE.

PAUL R. HERSHMAN, OF CHICAGO, ILLINOIS, ASSIGNOR TO THE MINERAL PRODUCTS COMPANY, OF NEW YORK, N. Y., A CORPORATION OF WEST VIRGINIA.

## PRODUCTION OF METALLIC COMPOUNDS FROM CARBIDS.

1,220,843.

Specification of Letters Patent. Patented Mar. 27, 1917.

No Drawing.

Application filed December 21, 1914. Serial No. 878,814.

*To all whom it may concern:*

Be it known that I, PAUL R. HERSHMAN, a citizen of the Empire of Austro-Hungary, residing in the city of Chicago, county of 5 Cook, State of Illinois, have invented certain new and useful Improvements in Production of Metallic Compounds From Carbids; and I do hereby declare the following to be a full, clear, and exact description of 10 the invention, such as will enable others skilled in the art to which it appertains to make and use the same.

The present invention is based upon the discovery that if aluminum carbid is heated 15 (preferably under pressure) to a sufficiently high temperature, it will, in decomposing, yield metallic aluminum. It has been found further that the reaction is facilitated by the presence of oxids, sulfids, or chlorids of 20 aluminum, or of some other suitable metal, such as copper, present in such proportions as to form with the aluminum the eutectic alloy of the two metals, that is to say, the alloy of definite composition and definite 25 physical properties having the lowest melting point of all the possible alloys of its constituent metals. Furthermore, the reduction is accomplished with additional facility in the presence of certain gases which do not 30 tend to interfere with the decomposition of the carbids or to reconstruct the carbids after decomposition; such gases being, for instance, hydrocarbons and particularly hydrogen, which latter seems to have a catalytic 35 effect in the general operation.

In carrying the invention into effect, I preferably charge the aluminum carbid, in a compact mass into an electric furnace of the vertical type, that is to say, a furnace 40 wherein the electric current traverses the charge from top to bottom. With the aluminum carbid of the charge may be associated small quantities (say 10%-20% by weight) 45 of aluminum oxid, aluminum chlorid, or aluminum sulfid. The several ingredients may be brought into union in any suitable way, as, for instance, by subjecting them to a mixing and kneading operation in a suitable mixer.

50 The reducing operation as hereinbefore indicated, is preferably carried on under pressure, and with the introduction of a suitable gas, admitted under pressure into the interior of the furnace. To this end, the 55 electric furnace should be fitted with a cover

securely held in place thereon, and the gas may be admitted into the interior of the furnace in any convenient way, as, for instance, through hollow arcing electrodes, if the furnace is of the electric arc type, or through a 60 hollow carbon resistance rod with a side entrance into the furnace chamber if the furnace is of the electric resistance type. The pressure developed in the electric furnace chamber may be determined by providing 65 the cover with a suitable vent, and the issuing gases may be burned as they take their exit from the vent; or, if desired, the issuing gas current may pass through a suitable 70 safety valve, which will hold the contents of the furnace automatically under regulable pressure. In practice, I have found superatmospheric pressure of from 10 to 15 pounds to the square inch to give satisfactory 75 results, but this pressure may be exceeded, due regard being had to such precautions as will prevent the pressure from rising beyond the limits of safety in any particular instance.

In some instances, the charge may be inserted, either in a compact mass or in briqueted form within an electric tube furnace, that is to say, a chamber of tubular form 80 whose walls are heated electrically. In practice, I have found when such a tube furnace 85 is brought to a temperature of 2200° C. that the charge begins to melt quickly, whereupon the temperature may be lowered somewhat (say to 2100° C.) with the production 90 of metallic aluminum.

When an oxid, chlorid, or a sulfid of another metal is employed, in admixture with the aluminum carbid, the ingredients thus added to the aluminum carbid should be present in such proportion that there will 95 result the eutectic alloy of the aluminum with the metal of the oxid, chlorid, or sulfid added, as hereinbefore specified. Thus, by way of example, the oxid, chlorid, or sulfid of copper, may be employed in such proportion as to produce the eutectic 100 alloy represented by 94.2% of aluminum and 5.8% of copper and which has a tensile strength of about 30,000 pounds.

What I claim is:

1. The method of producing metallic aluminum from aluminum carbid which comprises heating the carbid in the presence of gases which do not tend to interfere 105 with the decomposition of the carbids under 110

super-atmospheric pressure, and to a temperature sufficient to decompose the carbid and to produce metallic aluminum.

2. The method of producing metallic aluminum from aluminum carbid which comprises heating the carbid to a temperature of about 2200° C.

3. The method of producing metallic aluminum from aluminum carbid which comprises heating the carbid to a temperature of about 2200° C., in the presence of a small amount of a metal compound facilitating the decomposition.

4. The method of producing metallic aluminum from aluminum carbid which comprises heating the carbid with small quantities of an additional aluminum compound facilitating the decomposition to a temperature of about 2200° C. until the charge begins to melt and thereafter lowering the temperature to about 2100° C. for further effecting the decomposition of the carbid and the formation of aluminum.

5. The method of producing metallic aluminum from aluminum carbid which comprises heating the carbid in the presence of a gas containing hydrogen which does not tend to interfere with the decomposition of the carbids under superatmos-

pheric pressure, and to a temperature sufficient to decompose the carbid and to produce metallic aluminum.

6. The method of producing metallic aluminum from aluminum carbid which comprises heating the carbid admixed with a small amount of an additional aluminum compound other than the carbid, in the presence of gases which do not tend to interfere with the decomposition of the carbid under super-atmospheric pressure, and to a temperature sufficient to effect the decomposition of the carbids and the production of aluminum.

7. The method of producing metallic aluminum from aluminum carbid which comprises heating the carbid in the presence of gases which do not tend to interfere with the decomposition of the carbids under a super-atmospheric pressure of about ten to fifteen pounds to the square inch, and to a temperature sufficient to decompose the carbid and to produce metallic aluminum.

In testimony whereof I affix my signature, in presence of two witnesses.

PAUL R. HERSHMAN.

Witnesses:

M. AMES,  
M. A. BILL.